

## UNITED STATES PATENT OFFICE

1,955,892

## ARTIFICIAL LEATHER

Milton O. Schur, Berlin, N. H., assignor to Brown  
Company, Berlin, N. H., a corporation of MaineNo Drawing. Application January 11, 1932,  
Serial No. 586,091

4 Claims. (Cl. 91—68)

This invention relates to the manufacture of an artificial leather, and more especially one which can be produced at low cost and yet be serviceable as a shoe innersole stock, or for other purposes.

In making artificial leathers, one of the most inexpensive raw materials available for making the fibrous foundation is preliberated cellulose pulp, and more specifically wood pulp which can be converted into a waterlaid web on machinery of the papermaking type. When such a web is impregnated with rubber solutions of water-dispersed rubber, e. g., rubber latex, and then dried, it takes on leather-like properties to such an extent that it can serve for such purposes as shoe innersoles. Thus, the rubber-impregnated web is possessed of sufficient residual porosity to permit breathing of the foot and its constituent fibers are sufficiently bonded together to resist disintegration through the action of moisture and perspiration.

I have found that in making such artificial leathers, it is highly advantageous to use as the fibrous base a waterlaid web composed of a blend of both cellulose fibers like preliberated wood pulp and wool fibers. Aside from the fact that wool fibers lend themselves to web formation, especially when blended with cellulose fibers, and can take on rubber from rubber solutions or aqueous dispersions, wool fibers can be had on the market at a much lower cost than even wood pulps of the cheapest grade. For example, it is possible now to purchase wool cuttings or shoddies at as low as \$10 a ton, which is much lower than the current cost of even the cheapest grades of wood pulp. These wool cuttings or shoddies are sometimes made up of wool fibers of different colors, in which case they impart a pleasing variegation of the web, both in its raw and rubber-impregnated state. The wool fibers alone, however, do not conduce to waterlaid webs having a uniform texture, which result may, however, be had when cellulose fibers or the like are blended with the wool fibers in aqueous suspension and the mixed fibrous suspension is run off into a web on a suitable papermaking machine, e. g., a machine of the Fourdrinier or cylinder type.

The cellulose fibers used as raw material may be any one or a mixture of the well-known chemical wood pulps, e. g., sulphite or kraft pulp, either in bleached or unbleached condition. Preferably, however, a refined wood pulp of an alpha cellulose content of about 93% to 96% is employed, as such pulp leads to webs of greater absorptivity on a given papermaking machine.

Preliberated cellulose pulps other than wood pulp may be used when available, in lieu of part or all of the wood pulp, for instance the longer-fibered pulps derived from manila, sisal, ramie, or the like. The blend may contain various proportions of preliberated cellulose pulp and wool fiber, for instance a preponderant proportion of either. On the other hand, the use of more cellulose pulp than wool fiber is ordinarily to be preferred because of the uniform web texture attainable in such case without much trouble. For example, a blend of about 75% to 50% refined wood pulp and about 25% to 50% wool fiber has been found to yield an excellent web for use as an artificial leather base.

I shall now give a specific example of procedure which has been found to give an artificial leather eminently satisfactory for use as shoe innersole stock. I first prepare an aqueous fiber suspension in a beater engine made up of about 75% refined wood pulp of an alpha cellulose content of about 93% to 96% and about 25% wool shoddy, which may contain fibers of mixed colors. The beater should be operated in such a way as to effect a mixing of the fibers without much hydration or gelatinization of the wood pulp fraction, if a comparatively flexible artificial leather is desired; if a stiffer leather is in view, the wood fibers may be correspondingly hydrated.

The mixed aqueous fiber suspension is diluted with sufficient water to form a comparatively dilute and uniform fiber suspension, which is run off on a papermaking machine operated under conditions to deliver a dry web having a compactness of, say, about 40 and a basis weight of about 300. The compactness value is obtained by dividing the basis weight in pounds by the thickness in inches, and multiplying by the factor  $10^{-2}$ . The expression "basis weight" as known in papermaking circles represents the weight in pounds of 480 sheets whose dimensions are 24 x 36 inches, this being equivalent to 2880 square feet of sheet material. In other words, the compactness value really represents the weight of fiber per unit volume of sheet material.

The dried, raw web is then impregnated with a suitable latex composition, as by immersion in the composition, and then dried. No difficulty whatever is encountered in securing complete impregnation of the sheet, because it is comparatively porous. Preferably, the latex composition contains casein as a stiffening agent, and also lime, which latter compound serves to prevent migration of the rubber particles to the surface of the impregnated sheet during the drying operation.

It is desirable to add a slight amount of viscose to the latex composition, as the regenerated cellulose produced in the sheet during drying improves its characteristics. When viscose is present in the composition, boric acid is also preferably added along with the viscose to promote the regeneration of the cellulose from the viscose. The boric acid or its equivalent is added to the viscose without causing a gelling, and serves primarily to neutralize part of the alkali associated with the viscose. A suitable anti-oxidant, such as "Agerite White" is preferably added to the latex composition in order to improve the ageing qualities of the dried, rubber-impregnated sheet.

I do not herein claim as the invention the advantageous latex composition, as this subject matter is disclosed and claimed in my patent application Serial No. 541,959, filed June 3, 1931. The particular latex composition used as the impregnant may have a total solids content (i. e., rubber and non-rubber solids) of about 9% in the bath whereinto the raw web is dipped. When the impregnated sheet is dried, it contains about 20% to 25% added solids, and compares favorably with an artificial leather made entirely of a refined wood pulp base and impregnated with a similar latex composition to a much higher solids content. I present herewith a table showing the characteristics of the artificial leather of the present invention, alongside of one whose fibrous base consisted entirely of refined wood pulp of a compactness of about 30 and which imbibed about twice as much solids from a common latex composition used as the impregnant:

|                                      | New artificial leather | Artificial leather (100% refined wood pulp base) |
|--------------------------------------|------------------------|--------------------------------------------------|
| 40                                   |                        |                                                  |
| Solids added (% based on fiber)..... | 22                     | 40                                               |
| Thickness.....                       | .060                   | .072                                             |
| Stiffness, wide bend:                |                        |                                                  |
| With direction of sheet.....         | 650                    | 450                                              |
| Across direction of sheet.....       | 860                    | 590                                              |
| Stiffness, sharp bend:               |                        |                                                  |
| With direction of sheet.....         | 600                    | 580                                              |
| Across direction of sheet.....       | 675                    | 580                                              |
| Tack holding.....                    | 17                     | 17                                               |
| Internal ply adhesion.....           | 110+                   | 140                                              |

It is thus seen that in so far as concerns those properties such as stiffness, tack-holding ability, and internal ply adhesion, desired in innersoles, the new artificial leather compares quite favorably with a much more expensive artificial leather containing only refined wood pulp as the fibrous base, and far more added solids. The new artificial leather has lower tear resistance than the single ply artificial leather used as a basis of comparison, but this feature is not of great moment in such articles as inner soles, which do not undergo tearing stresses in use. Were a two-ply artificial leather, but otherwise similar to the standard of comparison appearing in the table, used as a basis of comparison, however, the new artificial leather would measure up with such a two-ply artificial leather, even in such respects as tear resistance.

One of the important advantages attending the use of wool fiber along with cellulose fiber in the furnish is that the web producible therefrom is much freer from wrinkles, cracks, or other surface blemishes than a web prepared from an all-cellulose fiber furnish, and accordingly the rubber-impregnated, artificial leather product into which the wool-containing web is converted as

a result of impregnation with a latex composition and drying presents a more perfect surface. This is evidently attributable to the resiliency of the wool fibers and the tendency of a web containing such fibers to recover from any localized denting or marring action which it undergoes during manufacturing operations. The fluffy kind of webs of low compactness which I fabricate as the foundations for artificial leather products are susceptible to becoming surface-blemished, especially when of high basis weight. Thus, at a basis weight of about 150 pounds and higher, such webs tend to acquire surface cracks and other blemishes, probably on account of their contact with the instrumentalities of the papermaking and impregnating machines, for instance the rolls and/or drying drums of these machines, and/or probably because of the tendency of the inner layers of a comparatively thick sheet to "pipe" or to crack when bent into a small arc. A web made from only a refined wood pulp and having a basis weight of 200 pounds and a compactness of 40 showed surface defects even though the smallest roll on the papermaking machine at the dry end did not exceed 4 inches in diameter. When the furnish contained 25% wool fibers, there was no evidence whatever of surface defects in a web of the same high basis weight and low compactness. Heretofore, in the manufacture of a 3-iron artificial leather (i. e., leather of a thickness of 3/48 inches) intended as for innersoles, it was found necessary to use at least two plies of web stock of a compactness of about 40, in order to realize a product of satisfactory appearance. The plies were superposed and bonded together after each had undergone impregnation with rubber independently to acquire the desired leather-like characteristics. If it is attempted to produce a similar artificial leather product from only a single ply of 300 pounds basis weight containing only cellulose fiber, it is found that the finished product is badly cracked on its surface and presents a distinctly inferior appearance. When, on the other hand, the furnish from which the web is prepared contains about 25% wool, it is found that a single-ply web can be properly fabricated at a basis weight of 300 pounds or even higher, and that such a web can serve as the complete base for an artificial leather innersole practically free from unsightly surface markings. Besides, it is more economical to work with a single ply of heavy weight, because it is sufficiently strong as it comes off the dry end of the paper machine, even at low compactnesses, say at a compactness of about 40, to resist rupture or breakage when processed as a continuous sheet and because the cost of laminating is eliminated.

It is noteworthy of mention that webs containing refined wood pulp of an alpha cellulose content of, say, about 93% to 96% are generally more absorptive and lead to artificial leathers of greater flexibility and suppleness than do unrefined pulps. If it is attempted to cheapen the furnish by substituting unrefined pulp for part or all of the refined wood pulp, the quality of the web is correspondingly impaired. It was only after considerable experimentation that wool fiber was established as being a component which would reduce the cost of the furnish and yet in certain important respects enhance the quality of the web and the ultimate artificial leather, particularly when the wool is used in proportion up to, say, about 40% to 50% of the dry weight of the entire fiber furnish.

I claim:

1. A rubber-impregnated, waterlaid web of fibers made up partly of cellulose fibers and partly of wool fiber, said web having a compactness not exceeding about 40, as determined by dividing its basis weight in pounds by its thickness in inches and multiplying by the factor  $10^{-2}$ , and a basis weight of at least about 150, but at the same time being substantially free from surface defects. 5 80
2. A dried, latex-impregnated, waterlaid web of fibers made up partly of substantially unhydrated wood pulp and partly of wool shoddy, said web having a compactness not exceeding about 15 40, as determined by dividing its basis weight in pounds by its thickness in inches and multiplying by the factor  $10^{-2}$ , and a basis weight of at least about 150, but at the same time being substantially free from surface defects. 90
- 20 3. A dried, latex-impregnated, waterlaid web of interfelted fibers made up largely of substantially unbeaten wood pulp having an alpha cel- 95

MILTON O. SCHUR.

100  
25  
30  
35  
40  
45  
50  
55  
60  
65  
70  
75  
105  
110  
115  
120  
125  
130  
135  
140  
145  
150